

June 24, 1924.

1,498,657

M. N. HURD

PORCELAIN ENAMELED TABLE TOP AND METHOD OF MAKING THE SAME

Filed Nov. 20. 1923



INVENTOR

M. N. Hurd  
by F. N. Barber  
attorney

## UNITED STATES PATENT OFFICE.

MARION N. HURD, OF FRANKFORT, INDIANA, ASSIGNOR TO INGRAM-RICHARDSON MANUFACTURING COMPANY, OF BEAVER FALLS, PENNSYLVANIA, A CORPORATION OF PENNSYLVANIA.

## PORCELAIN-ENAMELED TABLE TOP AND METHOD OF MAKING THE SAME.

Application filed November 20, 1923. Serial No. 675,972.

To all whom it may concern:

Be it known that I, MARION N. HURD, a citizen of the United States, residing at Frankfort, in the county of Clinton and State of Indiana, have invented new and useful Improvements in Porcelain-Enamelled Table Tops and Methods of Making the Same.

My invention relates to porcelain enamelled table-tops and methods of making the same. In the manufacture of table-tops of the class described and that variety thereof which has an inturned metal flange at the lower edge of the vertical flange surrounding the table-top, it has been customary to place porcelain enamel on the lower side of the said inturned metal flange. I have found that if the porcelain enamel be wiped off from the lower side of the said inturned flange before the porcelain enamel on the remainder of the table top is burnt or fired the bottom of the flange will be finished in better condition and the porcelain enamel burnt on the said vertical flange which surrounds the table top will not become cracked or broken in handling or use.

This will be better understood by reference to the accompanying drawings in which Fig. 1 is a perspective view of a table top, the view showing the under side of the table top; Fig. 2, is a sectional view showing a corner of a table top in its finished condition; Fig. 3, a sectional view through one edge of the table-top, showing the first step in the coating of the table-top; Fig. 4, a view similar to Fig. 3, showing the next step, and Fig. 5, a view similar to Fig. 4, showing the final step in the manufacture of the table-top.

Before the table-top has been coated with enamel it comprises a sheet metal structure having the horizontal top member 1, the vertical middle flange or member 2 surrounding the member 1 and connected thereto, and the inturned flange or member 3 connected to the lower edge of the member 2. The metal structure just described is covered with a prime coat 4 of clear or dark blue enamel and this coated structure is placed in an enameling furnace in which the enamel is burned on the said metal structure. The coat of enamel may cover the entire

structure as shown on Figs. 2, 3, 4 and 5. The structure is then covered on the upper surface of the member 1, the outer surface 55 of the member 2, and the lower surface of the member 3 with a coat 5 of porcelain enamel having the desired color as shown on Fig. 4. Then that part of the coat 5 lying beneath the coat 4 on the member 3 is wiped 60 off, leaving the appearance as shown on Fig. 5. The structure so coated is again placed in the enameling furnace and burned in the usual manner.

In the shipping or other handling of table-tops which have the coat 5 extending beneath the member 3, the coat 5 on the outer side of the member 2 often becomes cracked and broken, due to knocks or other injuries applied to the under side of the said flange 70 3. It is to be understood that the coat 5 is of a glassy nature and is quite brittle and that any checking or breaking of the enamel beneath the flange 3 would be very likely to be extended into the enamel on the outer 75 face of the member 2. The coat 4 of enamel on the bottom of the flange 3 is thin and is not liable to break as easily as white enamel which has a greater thickness.

It is common to lay the table-tops on 80 racks in the enameling furnace. If the table-top shown would be placed in the enameling furnace with the flange or member 3 downward and if this flange so coated is placed upon the usual racks therein, this 85 coat will become more or less marred during the enameling process.

It is thus seen that by removing the coat 5 from beneath the flange 3 or the coat 4 thereon, or by not applying the coat 5 to the 90 lower side of the flange 3 or the coat 4 thereon, I provide a porcelain enamel table-top whose enameled surface of the member 2 is not liable to become cracked or broken and that has the under surface of the flange 3 95 or the coat 4 thereon unmarred by rack marks.

Although the drawing shows but a single coat 5 of enamel on the prime coat 4, it is to be understood that there may and very often 100 are two, three or even four coats thereon, there being employed a sufficient number of coats to cover defects, but each coat is applied as the first coat 5 and is wiped off from

the lower surface of the prime coat 4 on the bottom of the flange 3 before each firing operation.

I claim—

- 5 1. In a table-top, a sheet-metal top member, a vertical sheet metal pendent flange member connected to the edge of the top member, an inturned flange member connected to the bottom of the pendent flange member, a ground coat of enamel on the sheet-members, and a porcelain enamel coat on the ground coat on the upper surface of the top member and of the pendent flange member, but not on the ground coat on the 10 under surface of the inturned flange member.
2. In a table-top, a sheet-metal top member, a vertical sheet metal pendent flange member connected to the edge of the top member, an inturned flange member connected to the bottom of the pendent flange member, and a porcelain enamel coat over the upper surface of the top member and of the pendent flange member, but not on the 15 ground coat on the under surface of the in-turned flange member.
- 20 3. The method of manufacturing an enameled sheet-metal table-top, which consists in making a sheet-metal top member with a

pendent flange connected to its edge and 30 with an inturned flange connected to the lower edge of the pendent flange, then coating the table-top with a ground coat of enamel, burning the same on the sheet metal, 35 providing the ground coat on the upper surface of the top member and the outer surface of the pendent member with a coat of porcelain enamel, and burning the latter on its supporting structure.

4. The method of manufacturing an 40 enameled sheet-metal table-top, which consists in making a sheet-metal top member with a pendent flange connected to its edge and with an inturned flange connected to the lower edge of the pendent flange, then coating 45 the table top with a ground coat of enamel, burning the same on the sheet-metal, coating the ground coat on the upper surface of the top member, the outer surface of the pendent flange, and the lower surface of the inturned flange with a coat of porcelain enamel, removing the latter coat from the latter flange, and burning the remaining portion of the porcelain enamel 50 coat on its supporting structure.

In testimony whereof, I hereunto affix my signature this 14th day of November, 1923.

MARION N. HURD.